

## UNITED STATES PATENT OFFICE

2,281,895

## LIGHT SENSITIVE MATERIAL

Gottlieb von Poser, Wiesbaden, and Maximilian  
Paul Schmidt, Wiesbaden-Biebrich, Germany

No Drawing. Application November 14, 1940, Se-  
rial No. 365,652. In Germany November 20,  
1939

25 Claims. (Cl. 95—7)

The present invention relates to light sensitive materials which may be used for photographic purposes.

It is known that the light-sensitiveness of such organic dyestuffs as change their color or bleach out on exposure to light may be enhanced by adding sensitizers to the dyestuffs. As such sensitizers there have been proposed, for instance, thiosinamine and anethole. By applying combinations of suitable dyestuffs with such sensitizers on paper or a similar support, light-sensitive materials are obtained which may be used for photographic purposes. Such light-sensitive materials, however, have hitherto not attained a great importance in view of the fact that the light-sensitiveness of the dyestuffs which in most cases is only very small is not sufficiently enhanced by the sensitizers so that the light-sensitive materials require too long times of exposure.

Now, we have found that the anthraquinone and the derivatives thereof are suitable sensitizers for the above mentioned light-sensitive layers containing organic dyestuffs. The derivatives which have a good solubility in water and are colorless or only feebly colored may be used with special advantage. Thus, for instance, the benzene nuclei of the anthraquinone may carry simple substituents such as alkyl groups, halogen atoms, carboxylic or sulfonic acid groups. Anthraquinone sulfonic acids and their water-soluble salts are particularly suitable. Above all beta-anthraquinone sulfonic acids, for instance, 2,7-anthraquinone disulfonic acid must be mentioned. 2-anthraquinone monosulfonic acid may also be used with good success. Instead of the anthraquinone or its derivatives there may be used the benzanthrone or the derivatives thereof, especially the benzanthrone sulfonic acids. The latter compounds, however, are not so effective as the anthraquinone compounds.

By means of the compounds used as sensitizers according to the present invention the light-sensitiveness of dyestuffs may be enhanced to a considerable extent, i. e. in general to a multiple of the light-sensitiveness obtained by sensitization of dyestuffs with known sensitizers. It is even possible, according to this invention, to sensitize dyestuffs, which per se are practically not sensitive to light, to such an extent that they show a great light-sensitiveness and may, consequently be used for photographic purposes.

The sensitizers used according to the present invention are preferably applied together with azo-dyestuffs, for instance, very simple azo-dyestuffs, such as amino-azobenzene or complicated

azo-dyestuffs, such as, disazo-dyestuffs, trisazo-dyestuffs or tetrokisazo-dyestuffs. The best results are generally obtained with monoazo-dyestuffs, especially such as contain one or several basic groups, preferably amino groups. There are also suitable triphenylmethane dyestuffs for instance, blue or violet triphenylmethane dyestuffs. When combined with the said sensitizers they very quickly turn yellow-green or green, respectively, on exposure to light. Oxazine dyestuffs such as Nile-blue or quinone dyestuffs such as Alizarinirisol D or Alizarinsaphirol B (see Schultz Farbstofftabellen 1931, Nos. 1,029, 1,196 and 1,187) and other water soluble dyestuffs will also be used. It may easily be ascertained by experiment whether and to which extent a dyestuff is suitable. For this purpose it is only necessary to add one of the sensitizers to a dilute dyestuff solution, to pour the solution on absorptive paper and to expose the latter half covered for a short time to arc or sun light or to another source of light emitting actinic light.

It is suitable to add to the dyestuffs considerable amounts of sensitizers. In some cases it is advantageous that the quantity of the sensitizer surpasses that of the dyestuff. In general it is advisable to add to the mixtures of dyestuffs and sensitizers an acid since in this manner the dyestuffs may often be brought into a form especially sensitive to light, as more fully described below.

The said combinations of dyestuffs and sensitizers may be applied in the form of their solutions on paper or any other support. Particularly good results have been obtained with these combinations in light-sensitizing foils, for instance, of regenerated cellulose or cellulose esters since on these supports the change of the dyestuffs occurs very rapidly. The light-sensitive layers thus obtained may be used for various purposes, for instance, for photometric researches since the changes of the dyestuffs are well visible and may, therefore, easily be observed. The layers may also be applied in the color photography or in heliographic printing for the preparation of prints. In the latter case there are advantageously used for the preparation of prints which shall be inspected dark, for instance, blue dyestuffs preferably those which entirely bleach out on exposure to light. For the preparation of so-called intermediate originals, however, which serve for the preparation of further prints, yellow dyestuffs are generally to be preferred.

A very important practical advantage of the said light-sensitive layers resides in the fact that they are of good stability in the dark. As is

known, this is not the case with other light-sensitive layers. Also with such light-sensitive layers which contain thiosinamine besides the dyestuffs it may often be observed that a change of the color or a decolorization takes place even when the material is stored in the dark.

In the preparation of prints by means of the new light-sensitive layers the fixation may be carried through in various ways according to the properties of the dyestuffs and sensitizers used. If in the case of a bleaching-out layer the sensitizer is soluble in a solvent in which the dyestuff does not dissolve, the sensitizer may be removed after exposure by washing out with the respective solvent. In many cases water may be used as solvent. If dyestuffs are used which per se are practically insensitive to light, stable prints may be obtained in this manner. Sometimes it is even possible to use for the fixation a liquid which dissolves the sensitizer and in which the dyestuff per se is likewise soluble. This method may be applied in case the dyestuff has substantive properties relative to the support or is rendered insoluble by a treatment with a mordant or a like operation.

In some cases the dyestuff differs in its form according to the pH-value of the layer. It often occurs that of the two forms which are generally of different color that one existing at a higher pH-value is not or hardly sensitive to light whereas that one existing at a lower pH-value is sensitive to light. The dyestuff is then used in the latter form, the fixation being performed in the dry way by treating the light-sensitive material with gaseous ammonia.

The following examples illustrate the invention:

(1) A film of regenerated cellulose is impregnated with a solution containing per liter of water 5 grams of the dyestuff prepared by coupling diazotized sulfanilic acid with beta-naphthol (Orange II Schultz Farbstofftabellen No. 189) 10 grams of phosphoric acid and 25 grams of 2.7-anthraquinone disulfonate of sodium. By exposing the orange-red film thus obtained to the light of an arc lamp, the coloration disappears in a few minutes. The film may, for instance, be used for photometric purposes. Films of similar properties may be obtained with the aid of azo-dyestuffs prepared by coupling of the following components: diazotized aniline and dimethylaniline (butteryellow O, Schultz Farbstofftabellen No. 28) 2.4-dimethoxy-1-diazobenzene and phenol, 4-chloro-1-diazobenzene-2-sulfonic acid and dibutylaniline, 4-chloro-1-diazobenzene-2-sulfonic acid and diphenylamine, 2.5-dichloro-1-diazobenzene-4-sulfonic acid and N-ethyl-N-benzyl-aniline, 1-diazo-4-(2'5'-dichlorobenzyl)-aniline and phenol. There may also be used diamine pure blue, diamine blue BB, half wool black K and benzo-brown B (see Schultz Farbstofftabellen Nos. 510, 513, 671 and 689).

(2) 10 grams of the dyestuff prepared by coupling 4-diazo-dimethylaniline and phenol, 20 grams of phosphoric acid and 20 grams of anthraquinone-beta-sulfonate of potassium are simultaneously dissolved in a mixture of 500 cc. of water and 500 cc. of alcohol. By impregnation with this solution paper or foils may be made sensitive to light.

(3) The azo-dyestuff obtained from diazotized 4-chloraniline and N-ethyl-N-cyclohexylaniline is sulfonated in known manner in order to impart to the dyestuff a good solubility in water. 25 grams of the sulfonated dyestuff, 20 grams of

phosphoric acid and 35 grams of 2.7-anthraquinone disulfonate of sodium are together dissolved in 1 liter of water. This solution is applied on one side of a superficially saponified foil consisting of acetyl cellulose. The bluish-red material is exposed under an original to the light of an arc lamp. At the places struck by the light the dyestuff bleaches out very quickly. The prints may be fixed by treating them with gaseous ammonia whereby the dyestuff assumes a light-yellow color stable to light. The prints obtained are suitable for further printing on diazo-photoprinting material. Instead of 2.7-anthraquinone sulfonate of sodium there may be used 40 grams of 1.4-dichloro-2-anthraquinone sulfonate of potassium. It is also possible to use instead of the dichloro compound, 1.2-diamino-anthraquinone-3-sulfonic acid in form of its sodium or potassium salt, the amino compounds, however, being in general less suitable on account of an intense coloration of their own.

(4) A cellulose hydrate foil is impregnated with a solution of 5 grams of erioglaucine (see Schultz, Farbstofftabellen 1931, No. 770) 10 grams of phosphoric acid and 20 grams of anthraquinone-2.7-disulfonate of sodium 1 liter of water. When exposed to light under an original the exposed parts change from blue to yellow-green. These exposed yellow-green parts absorb chemically active light better than the unexposed blue parts. Such a film may be used for the preparation of an intermediate original in case a positive shall be prepared on diazo-photoprinting paper from a negative. Like the erioglaucine there may be applied in a similar manner other triphenylmethane dyestuffs, for instance Acid Violet 4BN, Victoria-Blue 4R, Night-Blue or Water-Blue R, Naphthalene-Green V or Malachite-Green B. Also the oxazine dyestuff Nile Blue BX is likewise suitable (see Schultz, Farbstofftabellen Nos. 803, 793, 823, 816, 777, 754 and 1029).

(5) A cellulose-hydrate film is impregnated with a solution of 10 grams of the blue dyestuff obtained by coupling tetramethyldiaminodiphenylethylene with diazotized sulfanilic acid (see Dissertation of Karl Riener, Bonn, 1938) 15 grams of phosphoric acid and 20 grams of 2.6-anthraquinone-disulfonate of sodium. The film obtained has a good sensibility to light.

(6) The azo-dyestuff obtained by diazotization of 4-chloraniline-3-sulfonic acid and subsequent coupling with dibutylaniline is subsequently sulfonated in order to improve its solubility in water. A light-sensitive material is prepared by impregnating a cellulosehydrate film with a solution containing per liter of water 15 grams of the sulfonated dyestuff, 20 grams of phosphoric acid and 40 grams of the sodium salt of benzanthrone-sulfonic acid. The latter is obtained by introducing benzanthrone into 6 or 8 times the quantity of fuming sulfuric acid containing 20% of free sulfuric anhydride, the temperature of the mixture rising to about 60° C. and sulfonation taking place. When a test portion shows that the product obtained is entirely soluble in water, the whole is diluted with ice water and the sodium salt of benzanthrone-sulfonic acid is isolated by addition of sodium chloride. Instead of the benzanthrone-sulfonic acid the sulfonic acid of naphthanthraquinone prepared in an analogous manner may be used.

We claim:

1. Light sensitive material which consists of a sheet support carrying a colored layer which layer changes their shade on exposure to light

wherein the said layer comprises a dyestuff which is unstable to light and as a sensitizer a substance selected from the group consisting of anthraquinone and benzanthrone compounds.

2. Light sensitive material as claimed in claim 1 wherein the said dyestuff is water soluble.

3. Light sensitive material as claimed in claim 1 wherein the said dyestuff is an azo dyestuff.

4. Light sensitive material which consists of a sheet support carrying a colored layer which layer changes their shade on exposure to light wherein the said layer comprises a mono-azo dyestuff which is unstable to light and as a sensitizer a substance selected from the group consisting of anthraquinone and benzanthrone compounds.

5. Light sensitive material as claimed in claim 4 wherein the said mono-azo dyestuff contains a basic group.

6. Light sensitive material which consists of a sheet support carrying a layer which comprises a dyestuff capable of bleaching out on exposure of the layer to light and as a sensitizer a substance selected from the group consisting of water soluble anthraquinone and benzanthrone compounds.

7. Light sensitive material as claimed in claim 6 wherein the said dyestuff is a water soluble dyestuff.

8. Light sensitive material as claimed in claim 6 wherein the said dyestuff is an azo dyestuff.

9. Light sensitive material as claimed in claim 6 wherein the said dyestuff is a mono-azo dyestuff.

10. Light sensitive layer as claimed in claim 6 wherein the said dyestuff is a mono-azo dyestuff containing a basic group.

11. Light sensitive material which consists of a sheet support carrying a layer which comprises a dyestuff capable of bleaching out on exposure of the layer to light and as a sensitizer a substance selected from the group consisting of substantially colorless anthraquinone and benzanthrone compounds.

12. Light sensitive material according to claim 11 wherein the said dyestuff is a water soluble dyestuff.

13. Light sensitive material as claimed in claim 11 wherein the said dyestuff is an azo dyestuff.

14. Light sensitive material as claimed in claim 11 wherein the said dyestuff is a mono-azo dyestuff.

15. Light sensitive layer as claimed in claim

11 wherein the said dyestuff is a mono-azo dyestuff containing a basic group.

16. Light sensitive material which consists of a sheet support carrying a layer which comprises a dyestuff capable of bleaching out on exposure of the layer to light and as a sensitizer a substance selected from the group consisting of water soluble substantially colorless anthraquinone and benzanthrone compounds.

17. Light sensitive material according to claim 16 wherein the said dyestuff is a water soluble dyestuff.

18. Light sensitive material as claimed in claim 16 wherein the said dyestuff is an azo dyestuff.

19. Light sensitive material as claimed in claim 16 wherein the said dyestuff is a mono-azo dyestuff.

20. Light sensitive layer as claimed in claim 16 wherein the said dyestuff is a mono-azo dyestuff containing a basic group.

21. Light sensitive material which consists of a sheet support carrying a layer which comprises an azo dyestuff capable of bleaching out on exposure of the layer to light and as a sensitizer a water soluble substantially colorless anthraquinone derivative which contains a sulfo group as a substituent in an aromatic nucleus.

22. Light sensitive material which consists of a cellulose hydrate foil which is impregnated with a mixture comprising a mono-azo dyestuff capable of bleaching out on exposure of the layer to light and a water soluble substantially colorless anthraquinone derivative which contains a sulfo group as a substituent in an aromatic nucleus.

23. Light sensitive material which consists of a cellulose hydrate foil which is impregnated with a mixture comprising a mono-azo dyestuff capable of bleaching out on exposure of the layer to light and 2,7-anthraquinone disulfonic acid.

24. Light sensitive material which consists of a cellulose hydrate foil which is impregnated with a mixture comprising a mono-azo dyestuff capable of bleaching out on exposure of the layer to light and 2-anthraquinone sulfonic acid.

25. Light sensitive material which consists of a cellulose hydrate foil which is impregnated with a mixture comprising a mono-azo dyestuff capable of bleaching out on exposure of the layer to light and 1,4-dichloro-2-anthraquinone sulfonic acid.

GOTTLIEB VON POSER.  
MAXIMILIAN PAUL SCHMIDT.